

June 9, 1942.

C. D. COXE

2,286,064

AMMUNITION

Filed June 12, 1940

2 Sheets-Sheet 1



*Fig. 3*



INVENTOR  
Charles D. Coxe  
BY *George*  
*D. Verne Smythe*  
ATTORNEYS

June 9, 1942.

C. D. COXE

2,286,064

AMMUNITION

Filed June 12, 1940

2 Sheets-Sheet 2

Fig. 4



Fig. 5



Fig. 6



## UNITED STATES PATENT OFFICE

2,286,064

## AMMUNITION

Charles D. Coxe, Bridgeport, Conn., assignor to  
Remington Arms Company, Inc., a corporation  
of Delaware

Application June 12, 1940, Serial No. 340,004

2 Claims. (Cl. 148—12)

This invention relates to the manufacture of ammunition components from steel and particularly from a steel that has a precipitation hardenable alloy therein. In the embodiment disclosed, the use of the steel is shown as applied to a cartridge case of the conventional rimfire type, but it is to be distinctly understood that the invention may be applied to any type of cartridge case and for other ammunition components, such as for example, shot shell heads and center fire cartridge primer cups.

Brass is in almost universal use as a cartridge case because, as will be shown later, it is the only metal previous to the invention herein described that has satisfactorily met the requirements in such use in regard to cost, shaping, strength, corrosion resistance and extractability from the gun. Brass, however, has many disadvantages and much work and research have been expended in the search for a substitute which will still meet the desired requirements. Brass is expensive and cannot be used in combination with certain very desirable primers and/or powders, as it will season crack, corrode, and will also cause reactions rendering the primers and/or powders unstable. The matter of expense is of particular importance in the manufacture of the conventional rimfire cartridges. There have been many attempts to use steel or an alloy thereof, but such has never proven feasible. The other objects of the invention will appear from the following description and illustrations which, as stated before, are not intended to limit the use of the invention to the forms shown and described.

In the drawings:

Fig. 1 is a sectional view of a rimfire cartridge case with the clearance between the case and the chamber of the gun exaggerated, the bulging of the shell due to firing pressures and a split being also exaggerated.

Fig. 2 shows diagrammatically, by way of example, sectional views of five stages in the forming of a rimfire shell from a flat blank to the finished rimfire case.

Fig. 3 is an enlarged view of a rimfire shell in which the tapering due to the drawing operations has been exaggerated.

Fig. 4 is a graph showing the relation between the relative elongation and the yield point and tensile strength of a copper bearing alloy which has been reduced in size by cold rolling. Two sets of curves appear in the graph, one for the metal as rolled after normalizing and the second

after it has been reheated for four hours at 450° C.

Fig. 5 is a graph showing the relation between Brinell hardness and time of reheating of a copper alloy steel which has previously been normalized.

In Fig. 6 there appears a graph which shows the number of splits and extraction force required for various materials in various stages 10 of treatment, including the conventional brass case and a copper alloy steel treated in accordance with the present invention.

The purpose of a cartridge case is to be a container or carrier for the powder and the 15 priming mixture which initiates the combustion of the powder. The projectile is placed in the mouth of the cartridge case and is propelled from the barrel when the primer of the cartridge is struck by the firing pin, thereby igniting the 20 propellant powder. When in position in the gun, the shell is located in the chamber thereof which is closely matched with the size of the shell, the shell being properly sized in the course of manufacture so that it will fit into the chamber. It 25 is obvious, however, that a certain clearance will always be present between the outside of the case and the chamber. There is also a variation in the snugness of the fit of the case in the chamber and the relative roughness of the chambers in different guns, all of which affect the 30 operation of the cartridge and extraction thereof.

Referring to Fig. 1, in which a conventional rimfire shell is depicted, 10 represents the bolt of the gun which has been closed against the 35 head 11 of the case 12. The case 12 fits within the chamber 13 of the barrel 14 (shown fragmentarily). An extractor 15 of the conventional type engages the rim of the shell as it is pushed into the chamber 14. A suitable striker or firing 40 pin 22 is provided to strike the rim of the case 12 in which the priming mixture is placed. It is to be noted that Fig. 1 is a horizontal section and that the striker in the case of a rimfire shell contacts the case at or near the edge of the rim. 45 It is necessary that the material of the case have sufficient strength and a sufficiently high yield point so that upon the combustion of the propellant charge and under the high pressure developed thereby, that it will not be forced a substantial amount beyond this yield point, because when such happens, the sides of the shell will be bulged outwardly and will remain permanently in that position, as is shown at 16 in exaggerated form (Fig. 1). It is desirable, however, that 50 at the time of firing of the shell, it be resilient

enough so that it will spring outwardly and seal the chamber, and prevent the escape of gases from the chamber of the barrel. In the event that the pressure is such as to cause the yield point of the metal in the shell to be exceeded thereby, allowing too great a permanent deformation to take place, it is obvious that the bulging portions of the shell will tightly engage the side of the chamber 13. This bulging of the shell will require an unusually high extraction force, which in many instances causes the extractor 10 to pull through the rim or portion of the shell with which it engages as the bolt is moved backwardly, leaving the expended shell within the chamber and causing great inconvenience and difficult operation. Even if the extractor does engage the shell and withdraw it, an excessive force is required to operate the gun, which obviously is undesirable. It is seen, therefore, that the yield point of the metal bears an important relationship to the extraction force necessary to withdraw the shell and also to the sealing of the powder gases and prevention of the escape thereof through the mechanism of the gun and into the face of the operator. Such leakage of gas backwardly also detracts power from the propelling of the projectile through the barrel of the gun and is undesirable. In the high velocity rimfire cartridges of the present day, the powder pressures at the initial time of firing are in the vicinity of 18,000 pounds per square inch, and of the standard rimfire shells in the vicinity of 14,000 pounds per square inch. The ductility of the metal of the case must also be such that upon the firing thereof it will not split, such as has been indicated at 17 of Fig. 1.

Brass shells also have the disadvantage of developing season cracks, which is attributed to the dezincification of brass in the shell caused by elements in the powder and primer composition attacking the zinc.

As is seen in Fig. 6, the extraction force in pounds required for a brass shell is 5 pounds in a particular type of firearm, and it can also be seen that the test showed no splits for the brass.

In Fig. 2, A, B, C, D, E, five of the steps in the forming of the usual rimfire shell are shown, it being understood that any number of intermediate operations may be used or any type of shell or case may be formed similarly.

A is a cross section through a circular disc of metal. It is usual to both form the disc A from a strip of metal and at the same time pass it through a die by means of a punch, and cup it as shown in B of Fig. 2. By successive drawing operations, the shell and rimfire case are shaped until they reach the final form shown in E.

In Fig. 3 is shown an enlarged view of a finished rimfire shell in which, due to the drawing operations, the upper portion indicated at 18 has been reduced by about 41% through the working. The section at 19 has been reduced by about 35% and the section in the base 0%, or the base remains substantially the same thickness as the original. It is obvious that these amounts vary in accordance with the dies and process used and are not limited to those shown. It has been found by the heat treating process, hereinafter described, that an alloy steel containing a precipitation hardenable material may be made that will have the proper tensile strength and ductility to satisfactorily operate in a gun, and tests have shown that it will have practically the same performance characteristics as the brass, as far as extraction force and splits are concerned, as can

be seen in Fig. 6 for the copper alloy steel, treated. Hitherto, attempts to use steel shells have resulted in failure because they split upon firing or the extraction force has been so great as to make it impossible to use them. It has also been difficult to suitably draw and form the cartridge case from the strip of metal and still have it so that it will function in the chamber of a gun. By the use of a copper bearing alloy steel, it has been found that it may be heat treated in the manner about to be described, and a successful cartridge case produced thereby.

In the heat treatment of a steel, it is said to be "normalized" after it has been brought to a temperature around or above 700° C., and then allowed to cool in air. It might also be cooled by quenching to hasten the cooling, or be allowed to remain in the furnace for a length of time, either of which will result in a different grain structure of the metal than when it is cooled in air, depending upon the percent of carbon in the steel or other alloying elements. When copper or other alloy making the steel precipitation hardenable, such as columbium, beryllium or titanium, is added to the steel, the steel may be heated to 700° C., preferably 800° to 900° C., at which time the copper goes into solid solution in the iron; then, upon cooling at a moderate rate such as in air, the copper stays in the solid solution. These temperatures are for copper as the precipitation hardenable element, and are not necessarily for the others. This may be termed "solution heat treating." If then the article be subjected to a heat of between 400° and 616° C. and held at that temperature for a period of from 16 hours to 10 minutes, respectively, as will be explained later, the copper which is in the solid solution will tend to precipitate out of the solution, whether or not this is complete not being known at present. However, it does have a very decided effect upon the metal. The copper is thrown out of the solution into a critically dispersed form, which may or may not be a precipitation, on reheating to a temperature that gives sufficient atomic mobility to allow the change. There is a possibility that some recrystallization will occur at the higher temperatures, but such is immaterial. This last heat treatment is known as "precipitation hardening." The tensile and yield strengths of steels that have not been cold shaped before the precipitation hardening are raised somewhat and the ductility decreased slightly. The graphs of Figs. 4 and 5, representing work of Cyril S. Smith and Earl W. Palmer, are copyrighted by the American Institute of Mining and Metallurgical Engineers and are used with the permission of that Institute. As may be seen by referring to Fig. 4, the yield point is raised from approximately 48,000 pounds per square inch to 68,000 pounds per square inch in a copper alloy steel of the composition indicated when 0% reduction by cold rolling has taken place. The percentage elongation in 2 inches, which is an indication of the ductility, is seen to fall from approximately 28% to 24%. However, if cold shaping or working takes place before the last heat treatment, such as occurs in the drawing of the shell, a very decided effect on the condition of the steel is produced by the cold working and precipitation hardening, it being necessary that the solution heat treating have taken place before the cold shaping.

Referring to Fig. 4 again, it is seen that with 41% reduction by cold shaping, that the yield point of the normalized or solution heat treated

steel is increased to 108,000 pounds per square inch, and that the ductility is reduced to about 3%. Upon reheating the cold shaped piece for 4 hours at 450° C., it is to be noted that the yield point remains substantially the same, and yet the percentage elongation is raised to about 12½%.

This puts the formed steel case in condition such that it may be satisfactorily used in a firearm because the yield strength has been increased to such a point that permanent deformation will not take place to any appreciable extent, thereby causing difficult extraction, nor will the shell split due to brittleness or lack of ductility thereof. The period of time which it is necessary to reheat for precipitation hardening the steel component depends upon the temperature and probably the degree of work hardening. In Fig. 5 it may be seen that if a temperature of 600° C. be used for a normalized copper alloy steel of the composition indicated, that the maximum Brinell hardness is reached in approximately 15 minutes, whereas if 450° C. be employed the maximum Brinell hardness is reached at some time between 16 and 64 hours, this Brinell hardness being slightly greater.

It is to be understood that the temperature used will depend upon the time the component is subjected thereto and should be a time temperature cycle wherein no or little recrystallization takes place. It has been found that a shell may be placed into a heat treating furnace and, when the shell reaches 616° C. in a period of 10 minutes, that satisfactory results will be obtained. If higher temperatures are used, a much shorter time of treatment must be employed or substantial recrystallization will take place, and the results will not be satisfactory.

Referring to Fig. 3, it is seen that in a conventional rimfire cartridge there is a much larger reduction of the wall near the mouth than there is near the lower part, and that in the base there is substantially no reduction. In the example shown, this is 41% near the mouth, 35% at the lower part of the wall, and 0% at the base. By referring to Fig. 4, it is noted that when the blank or cup is subjected, first, to a normalizing treatment, then is cold shaped, and then is reheated for the purpose of precipitation hardening, that at the mouth, the copper alloy steel as indicated in Fig. 4 will have a yield strength in the vicinity of 108,000 pounds per square inch and that the elongation will be about 12½%. At point 19 of the shell, the yield strength will be in the vicinity of 103,000 pounds per square inch, and the elongation about 13½%. In the base, the yield strength will be about 48,000 pounds per square inch, and the elongation about 24%. These figures are for purposes of explanation only and relate to the copper steel shown in Fig. 4 and not to the preferred alloys to be used. The wall therefore has sufficient strength and ductility produced by the cold working and precipitation hardening to withstand the firing pressures. It is also to be noted that the base is sufficiently soft so that the impact of the firing pin will be properly transmitted to the primer mixture, the strength at this point being immaterial because it is backed up by the bolt and does not receive the same forces that the case does near the mouth and along the wall. The advantage of such a distribution of strength and ductility in a cartridge case is obvious from the foregoing in that a shell with a wall that is of the proper strength

and characteristics is combined with a base having the desired properties.

During the cold shaping process of a rimfire shell, such as shown in Fig. 3, considerable strain is set up at the bend portion of the rim, which serves to work harden to a slight extent in this particular area. The heat treating temperature serves to relieve the stresses at this point, which also assists the sensitivity characteristics of the shell because the priming mixture is contained in the rim.

Referring now to Fig. 6, various types of shells have been tested and a comparison indicated. For brass, extraction force was found to be in the neighborhood of 5 pounds and no splits were recorded. The copper alloy steel after normalizing and drawing gave about 50% splits and 5 pounds extraction force. The same copper alloy steel upon the precipitation hardening treatment gave 0% splits and 5 pounds extraction force, which is substantially identical to the brass. It is preferable to use an alloy steel that has carbon in a low amount, not over .50% and preferably .10% or under. In order to strengthen or give desirable properties to the steel, any of the following elements singly or in combination in the amounts indicated may be used.

Nickel—not over 5.00%  
30 Silicon—not over 5.00%, preferably 0% to 1.50%  
Manganese—not over 3.00%, preferably 0.20% to 2.00%

Molybdenum—not over 1.00%, preferably less than 0.50%  
35 Chromium—not over 5.00%, preferably 0% to 2.00%

Vanadium—0% to 1.00%,  
or other alloying elements in such proportion  
40 as will increase the strength of the steel without  
so lowering the ductility as to make it impos-  
sible to fabricate. The phosphorus should be  
not over .50% and preferably under .25%. The  
copper in the steel should be not over 5.00% and  
preferably under 3.00%. As an example, the  
following steels have been found to be satis-  
factory:

No. 1

|            | Per cent    |
|------------|-------------|
| Carbon     | .08         |
| Manganese  | .50         |
| Silicon    | .10         |
| Nickel     | 2.00        |
| Phosphorus | maximum .04 |
| Sulphur    | do .04      |
| Copper     | 1.00        |

No. 2

|            | Per cent    |
|------------|-------------|
| Carbon     | .08         |
| Manganese  | .40         |
| Nickel     | 1.00        |
| Copper     | 1.30        |
| Molybdenum | .20         |
| Phosphorus | maximum .04 |
| Sulphur    | do .04      |

It is to be understood, however, that the invention is not limited to these two alloys, but that they are cited merely as examples of some that have proven to be satisfactory. The use of any of the alloying elements above mentioned or their equivalents or combinations thereof in a steel which will produce a yield point of substantially 50,000 pounds per square inch or more in the normalized steel and which renders the

steel capable of being precipitation hardened falls within the scope of the invention, the precipitation hardening serving to keep the yield strength of the cold shaped sections substantially constant and to increase the ductility so that the shell will function satisfactorily. It has been found that the best results are obtained with an alloy steel in which the copper is in excess of 0.5% and preferably between 1 and 2%. The shell is heated at some point, C or before of Fig. 2, to about 700° C. and preferably 800° to 900° C., and is maintained at this temperature for a sufficient time to permit the copper to go into solid solution in the iron. The component is then allowed to cool at moderate rate, such as in air or room temperature, this being fast enough to prevent any substantial precipitation of the copper from solid solution. The shell is then worked into a form such as in D of Fig. 2 so that the material of the walls of the shell receive cold working such as shown in Fig. 3, causing work hardening of the portions indicated. The shell in this condition, due to the increase in yield point, will probably have a low extraction force, as shown in Fig. 6, but, due to the lack of ductility, a large percentage of splits will take place. At this point or at D the shell is subjected to a temperature preferably between 400° and 616° C. and held there from between 16 hours to 10 minutes as indicated generally by Fig. 5, and preferably 450° to 500° C. for 4 hours. This gives the required ductility with only a slight change in the yield point or elastic limit, because the simultaneous precipitation hardening due to copper content will compensate for the loss in yield strength which ordinarily accompanies the heating of cold worked steel. It is to be noted that the graph of Fig. 5 is for illustrative purposes only and does not necessarily represent the preferred metal to be used. As a specific example, either steel 1 or 2, composition of which is set forth above, after step B, Fig. 2, is annealed at 620° C. to facilitate the drawing operation of step C of Fig. 2. After step C, the shell is heated at 870° C. for 1/2 hour and then air cooled. After step E, Fig. 2, the shell is heated to 450° C. for 4 hours and will then give the results substantially as shown in Fig. 6 in which the extraction force will be around 5 pounds and there will be no 50 splits.

It is to be understood that the annealing step is not essential nor is the normalizing or solution heat treating at 870° C., providing the steel can be properly drawn without cracking or undue wear and strain of the dies, and the normalizing is not necessary if, in the manufacture of the shell from which the component is cut, the sheet was so processed as to place the copper in solid solution in the iron.

10 5 If desired, the steel may be plated with copper or other rust inhibiting material placed thereon.

It is evident from the foregoing description that a method has been evolved and a novel 15 ammunition component produced that is superior in many ways to those in present day use. As the invention is believed to be the first time that a satisfactory steel ammunition component and method of producing the same has been provided, it is not limited to the details and composition shown herein, described in the drawings and illustrated, but is to be construed broadly as covering all equivalent devices and processes falling within the scope of the appended 20 claims.

25 What is claimed is:

1. In the manufacture of a cartridge shell, the 30 method which comprises providing a disc of low carbon steel containing a precipitation hardenable element; cold shaping said disc into a head of substantially the thickness of said disc and a body integral with said head which decreases in wall thickness toward the open end thereof; and, precipitation hardening the shell thus 35 formed, whereby is secured a maximum ductility in said head and an increasing yield strength toward the mouth of said body.

2. In the manufacture of rimfire cartridge 40 shells, the method which comprises providing a disc of low carbon steel containing copper in a state of solid solution, cold working said disc to form therefrom a cartridge shell comprising a head of substantially the thickness of said disc and a body of lesser thickness joined to said head by an integral folded hollow rim, and subsequently precipitation hardening the shell thus 45 formed to increase the ductility of the metal without material decrease in the yield strength of the metal.

CHARLES D. COXE.